# EUROPEAN PATENT APPLICATION

(11) **EP 4 239 094 A1**
(43) Date of publication of application: **06.09.2023**
(21) Application number: 21886102.9
(22) Date of filing: 22.10.2021
(51) Int. Cl.: C22C 38/00, C22C 38/60, H01F 1/14

(54) **SOFT MAGNETIC IRON**

(30) Priority: 29.10.2020 JP 2020181788
(71) Applicant: JFE Steel Corporation, Tokyo 100-0011 (JP)
(72) Inventor: ICHIMIYA, Katsuyuki, Tokyo 100-0011 (JP); NAKASHIMA, Koichi, Tokyo 100-0011 (JP); IMANAMI, Yuta, Tokyo 100-0011 (JP)
(74) Representative: Hoffmann Eitle
(86) International application number: PCT/JP2021/039162
(87) International publication number: WO 2022/091984

(57) **Abstract**

Provided is a technique that can achieve both magnetic properties and machinability by cutting at a high level, which has been impossible with only the conventional techniques of improving the machinability by cutting using MnS or the like. A soft magnetic iron comprises a chemical composition containing, in mass%, C: 0.02 % or less, Si: 0.15 % or less, Mn: 0.01 % or more and 0.50 % or less, P: 0.002 % or more and 0.020 % or less, S: 0.001 % or more and 0.050 % or less, Al: 0.05 % or less, N: 0.0100 % or less, and Se: 0.001 % or more and 0.30 % or less, with a balance consisting of iron and inevitable impurities.

## Description

### TECHNICAL FIELD

The present disclosure relates to a soft magnetic iron having excellent machinability by cutting and magnetic properties.

### BACKGROUND

Resource and energy saving is needed worldwide for global environment protection in recent years. In the field of electrical machinery, efficiency enhancement and downsizing are actively promoted with the aim of saving energy. Hence, electrical parts used in automobiles and the like are required to be more power-saving and be improved in the response speed to external magnetic fields.

Pure iron-based soft magnetic iron is typically used as material that easily responds to external magnetic fields. For such soft magnetic iron, a steel material having a C content of approximately 0.01 mass% or less is used. Usually, the steel material is hot rolled and then subjected to wiredrawing and the like to obtain a steel bar, and the steel bar is subjected to forging, cutting work, and the like to produce electrical parts.

It is known that, in parts machining, soft ferrite single phase contained in soft magnetic iron has very poor workability of cutting. This makes it increasingly important to provide soft magnetic iron excellent in not only magnetic properties but also workability.

For example, JP 2007-51343 A (PTL 1) discloses a technique of producing a soft magnetic steel material excellent in magnetic properties and machinability by cutting by controlling the size and number of MnS precipitates dispersed in steel.

JP 2007-46125 A (PTL 2) discloses a technique for a soft magnetic steel material excellent in cold forgeability, machinability by cutting, and magnetic properties by controlling the size and density of FeS precipitates.

### CITATION LIST

### Patent Literature

PTL 1: JP 2007-51343 A
PTL 2: JP 2007-46125 A

### SUMMARY

### (Technical Problem)

The techniques described in PTL 1 and PTL 2 each improve the machinability by cutting by the effect of MnS or FeS alone. However, increasing such precipitates (MnS or FeS) is likely to cause degradation in magnetic properties. There is thus a technical limit to achieving both magnetic properties and machinability by cutting at a higher level.

It could therefore be helpful to provide a technique that can achieve both magnetic properties and machinability by cutting at a high level, which has been impossible with only the conventional techniques of improving the machinability by cutting using MnS or the like.

### (Solution to Problem)

Upon careful examination, we newly discovered that the use of MnSe can improve the machinability by cutting without degradation in magnetic properties.

The present disclosure is based on this discovery and further studies. We thus provide:
1. A soft magnetic iron comprising a chemical composition containing (consisting of), in mass%, C: 0.02 % or less, Si: 0.15 % or less, Mn: 0.01 % or more and 0.50 % or less, P: 0.002 % or more and 0.020 % or less, S: 0.001 % or more and 0.050 % or less, Al: 0.05 % or less, N: 0.0100 % or less, and Se: 0.001 % or more and 0.30 % or less, with a balance consisting of iron and inevitable impurities.
2. The soft magnetic iron according to 1., wherein the chemical composition further contains, in mass%, one or more selected from the group consisting of Cu: 0.20 % or less, Ni: 0.30 % or less, Cr: 0.30 % or less, Mo: 0.10 % or less, V: 0.02 % or less, Nb: 0.02 % or less, and Ti: 0.03 % or less.
3. The soft magnetic iron according to 1. or 2., wherein the chemical composition further contains, in mass%, one or more selected from the group consisting of Pb: 0.30 % or less, Bi: 0.30 % or less, Te: 0.30 % or less, Ca: 0.0100 % or less, Mg: 0.0100 % or less, Zr: 0.200 % or less, and REM: 0.0100 % or less.

### (Advantageous Effect)

It is thus possible to provide a pure iron-based soft magnetic iron having excellent magnetic properties and machinability by cutting.

### DETAILED DESCRIPTION

A pure iron-based soft magnetic iron according to an embodiment of the present disclosure will be described below.

First, the reasons for limiting each component in the chemical composition of the pure iron-based soft magnetic iron will be described below. Herein, "%" representing the content of each component element is "mass%" unless otherwise stated.

### C: 0.02 % or less

If the C content is more than 0.02 %, the iron loss property degrades significantly due to magnetic aging. The C content is therefore limited to 0.02 % or less. If the C content is less than 0.001 %, the effect on the magnetic properties is saturated. Moreover, reducing the C content to less than 0.001 % requires higher refining costs. Accordingly, the C content is preferably 0.001 % or more. The C content is preferably in the range of 0.001 % or more and 0.015 % or less. The C content is more preferably in the range of 0.001 % or more and 0.010 % or less.

### Si: 0.15 % or less

Si is an element effective as a deoxidizing element. If the Si content is more than 0.15 %, ferrite hardens, and the cold workability decreases. Accordingly, although Si may be contained, its content is 0.15 % or less. The Si content is preferably 0.10 % or less. The Si content may be 0 %.

### Mn: 0.01 % or more and 0.50 % or less

Mn is an element that is not only effective in strength improvement by solid solution strengthening but also effective in improvement of machinability by cutting as a result of MnS, which is formed by combination of Mn and S, and MnSe, which is formed by combination of Mn and Se, dispersing in the steel. Accordingly, the Mn content is 0.01 % or more. If the Mn content is excessively high, the magnetic properties degrade. The Mn content is therefore 0.50 % or less. The Mn content is preferably 0.05 % or more. The Mn content is preferably 0.40 % or less. The Mn content is more preferably 0.15 % or more. The Mn content is more preferably 0.35 % or less.

### P: 0.002 % or more and 0.020 % or less

P has considerable solid solution strengthening ability even when added in a relatively small amount. To achieve this effect, the P content is 0.002 % or more. If the P content is excessively high, the cold workability is impaired. Accordingly, the upper limit is 0.020 %. The P content is preferably in the range of 0.002 % or more and 0.015 % or less.

### S: 0.001 % or more and 0.050 % or less

S forms MnS in the steel to contribute to improved machinability by cutting. To achieve this effect, the S content needs to be 0.001 % or more. If the S content is more than 0.050 %, the cold workability degrades. Accordingly, the S content is 0.001 % or more and 0.050 % or less. The S content is preferably 0.005 % or more. The S content is preferably 0.045 % or less. The S content is more preferably 0.010 % or more. The S content is more preferably 0.040 % or less.

### Al: 0.05 % or less

Al combines with N in the steel to form fine AlN. Such fine AlN hinders the growth of crystal grains and causes degradation in magnetic properties. The Al content therefore needs to be 0.05 % or less. The Al content is preferably 0.010 % or less, and more preferably 0.005 % or less. The Al content may be 0 %.

### N: 0.0100 % or less

If the N content is more than 0.0100 %, the cold workability and the magnetic properties degrade. Accordingly, the upper limit is 0.0100 %. The N content is preferably 0.0015 % or more. The N content is preferably 0.0090 % or less. The N content may be 0 %.

### Se: 0.001 % or more and 0.30 % or less

Se combines with Mn in the steel to form MnSe. This has the effect of improving the machinability by cutting. To achieve this effect, the Se content needs to be 0.001 % or more. If the Se content is more than 0.30 %, the magnetic properties and the castability degrade. Accordingly, the upper limit is 0.30 %. The Se content is preferably in the range of 0.001 % or more and 0.10 % or less. The Se content is more preferably in the range of 0.001 % or more and 0.05 % or less.

The basic components according to the present disclosure have been described above. The balance other than the foregoing components consists of Fe and inevitable impurities. The chemical composition may optionally further contain one or more of the following elements as appropriate:
Cu: 0.20 % or less,
Ni: 0.30 % or less,
Cr: 0.30 % or less,
Mo: 0.10 % or less,
V: 0.02 % or less,
Nb: 0.02 % or less, and
Ti: 0.03 % or less.

Cu, Ni, and Cr contribute to higher strength mainly by solid solution strengthening. To achieve this effect, the content of each element is preferably 0.01 % or more. If the content is excessively high, the magnetic properties degrade. Accordingly, the upper limits of the contents of Cu, Ni, and Cr are preferably 0.20 %, 0.30 %, and 0.30 %, respectively.

Mo, V, Nb, and Ti contribute to higher strength mainly by strengthening by precipitation. To achieve this effect, the contents of Mo, V, Nb, and Ti are preferably 0.001 % or more, 0.0001 % or more, 0.0001 % or more, and 0.0001 % or more, respectively. If the content of each element is excessively high, the magnetic properties degrade. Accordingly, the upper limits of the contents of Mo, V, Nb, and Ti are preferably 0.10 %, 0.02 %, 0.02 %, and 0.03 %, respectively.

The chemical composition according to the present disclosure may further contain one or more of the following elements:
Pb: 0.30 % or less,
Bi: 0.30 % or less,
Te: 0.30 % or less,
Ca: 0.0100 % or less,
Mg: 0.0100 % or less,
Zr: 0.200 % or less, and
REM: 0.0100 % or less.

Pb, Bi, Te, Ca, Mg, Zr, and REM are elements that contribute to improved machinability by cutting. To achieve this effect, the Pb content is preferably 0.001 % or more, the Bi content is preferably 0.001 % or more, the Te content is preferably 0.001 % or more, the Ca content is preferably 0.0001 % or more, the Mg content is preferably 0.0001 % or more, the Zr content is preferably 0.005 % or more, and the REM content is preferably 0.0001 % or more. If the content of each element is excessively high, the magnetic properties degrade. Accordingly, the Pb content is preferably 0.30 % or less, the Bi content is preferably 0.30 % or less, the Te content is preferably 0.30 % or less, the Ca content is preferably 0.0100 % or less, the Mg content is preferably 0.0100 % or less, the Zr content is preferably 0.200 % or less, and the REM content is preferably 0.0100 % or less.

The components other than the above in the chemical composition according to the present disclosure are Fe and inevitable impurities.

A preferred method of producing the pure iron-based soft magnetic iron according to the present disclosure will be described below.

Molten steel having the chemical composition described above is obtained by a smelting method such as a typical converter or electric furnace, and subjected to typical continuous casting or blooming to yield a steel material. The steel material is then optionally heated, and then subjected to hot rolling such as billet rolling and/or bar/wire rolling etc. to obtain a soft magnetic iron. The heating conditions and the rolling conditions are not limited, and may be determined as appropriate depending on the material properties required. For example, microstructure control is performed so as to be advantageous for subsequent forging, machining, etc. for forming parts. Since the soft magnetic iron according to the present disclosure has excellent workability of cutting, the shape of the soft magnetic iron is preferably any of a bar, a rod, and a wire, which are mainly used in applications involving cutting work.

The content of each element can be determined by the method for spark discharge atomic emission spectrometric analysis, X-ray fluorescence analysis, ICP optical emission spectrometry, ICP mass spectrometry, combustion method, etc.

The other production conditions may be in accordance with typical steel material production methods.

### EXAMPLES

Examples according to the present disclosure will be described below. The presently disclosed technique is, however, not limited to the examples below.

Steels having the chemical compositions shown in Table 1 were each obtained by smelting, then subjected to hot forging at approximately 1200 °C, and then subjected to annealing treatment at 950 °C to produce a steel bar of 25 mm in diameter. For each obtained steel bar, the magnetic properties, the cold workability, and the machinability by cutting were evaluated by the following methods. The evaluation results are shown in Table 2.

**Table 2**

| Steel sample ID | Magnetic properties | | | Cold workability | Machinability by cutting | Remarks |
|---|---|---|---|---|---|---|
| | Magnetic flux density at 100A/m (T) | Magnetic flux density at 300A/m (T) | Coercive force (A/m) | Critical upset ratio to crack initiation (%) | Flank wear (µm) | |
| A | 1.234 | 1.521 | 50.2 | 63.5 | 20.2 | Example |
| B | 1.275 | 1.581 | 48.9 | 59.1 | 29.5 | Example |
| C | 1.254 | 1.561 | 45.1 | 63.6 | 22.2 | Example |
| D | 1.217 | 1.533 | 47.2 | 63.4 | 25.7 | Example |
| E | 1.216 | 1.540 | 52.6 | 55.8 | 27.4 | Example |
| F | 1.210 | 1.522 | 47.9 | 60.7 | 29.4 | Example |
| G | 1.262 | 1.567 | 46.2 | 59.1 | 25.5 | Example |
| H | 1.204 | 1.513 | 45.3 | 58.2 | 26.7 | Example |
| I | 1.249 | 1.540 | 48.1 | 62.2 | 21.7 | Example |
| J | 1.232 | 1.526 | 51.9 | 60.3 | 21.0 | Example |
| K | 1.217 | 1.531 | 48.5 | 56.0 | 22.3 | Example |
| L | 1.211 | 1.506 | 53.9 | 55.2 | 29.1 | Example |
| M | 1.109 | 1.392 | 84.8 | 65.8 | 29.5 | Comparative Example |
| N | 1.272 | 1.596 | 71.6 | 60.9 | 42.0 | Comparative Example |
| O | 1.280 | 1.575 | 74.9 | 56.2 | 20.2 | Comparative Example |
| P | 1.264 | 1.565 | 45.9 | 42.2 | 24.7 | Comparative Example |
| Q | 1.244 | 1.560 | 81.3 | 65.8 | 25.1 | Comparative Example |
| R | 1.178 | 1.421 | 69.1 | 50.1 | 28.9 | Comparative Example |
| S | 1.239 | 1.546 | 81.4 | 46.7 | 26.5 | Comparative Example |
| T | 1.223 | 1.520 | 51.4 | 56.2 | 28.6 | Example |

Table 2(cont'd)

| Steel sample ID | Magnetic properties | | | Cold workability | Machinability by cutting | Remarks |
|---|---|---|---|---|---|---|
| | Magnetic flux density at 100A/m (T) | Magnetic flux density at 300A/m (T) | Coercive force (A/m) | Critical upset ratio to crack initiation (%) | Flank wear (µm) | |
| U | 1.273 | 1.606 | 74.5 | 50.9 | 21.4 | Comparative Example |
| V | 1.106 | 1.390 | 79.8 | 65.1 | 26.7 | Comparative Example |
| W | 1.093 | 1.377 | 74.3 | 58.4 | 26.2 | Comparative Example |
| X | 1.139 | 1.426 | 75.8 | 64.6 | 27.3 | Comparative Example |
| Y | 1.133 | 1.427 | 79.5 | 45.8 | 29.8 | Comparative Example |
| Z | 1.113 | 1.404 | 82.7 | 47.5 | 23.7 | Comparative Example |
| AA | 1.183 | 1.458 | 89.8 | 48.8 | 20.2 | Comparative Example |
| AB | 1.172 | 1.457 | 81.4 | 48.1 | 26.0 | Comparative Example |
| AC | 1.099 | 1.399 | 75.1 | 45.3 | 23.7 | Comparative Example |
| AD | 1.108 | 1.401 | 74.9 | 45.9 | 27.7 | Comparative Example |
| AE | 1.160 | 1.451 | 76.9 | 43.1 | 22.8 | Comparative Example |
| AF | 1.171 | 1.444 | 71.9 | 47.7 | 22.4 | Comparative Example |
| AG | 1.155 | 1.443 | 72.8 | 46.0 | 21.9 | Comparative Example |
| AH | 1.157 | 1.439 | 74.6 | 45.6 | 24.0 | Comparative Example |
| AI | 1.131 | 1.406 | 75.0 | 45.3 | 22.7 | Comparative Example |
| AJ | 1.226 | 1.531 | 55.1 | 58.7 | 37.2 | Comparative Example |
| AK | 1.234 | 1.539 | 54.3 | 60.3 | 38.4 | Comparative Example |
| AL | 1.209 | 1.527 | 52.7 | 56.9 | 28.8 | Example |
| AM | 1.212 | 1.529 | 55.1 | 59.5 | 27.6 | Example |
| AN | 1.165 | 1.419 | 68.5 | 48.2 | 27.2 | Comparative Example |

### [Magnetic properties]

The magnetic properties were measured in accordance with JIS C 2504. In detail, a ring-shaped test piece was collected from the steel bar (material), and subjected to magnetic annealing of holding at 750 °C for 2 h. After this, an excitation winding (primary winding: 220 turns) and a detection winding (secondary winding: 100 turns) were made around the ring-shaped test piece for testing. The magnetic flux density was determined by measuring the B-H curve using a DC magnetizing measurement device. Specifically, the respective magnetic flux densities at 100 Aim and 300 Aim in a magnetization process with a peak magnetic field of 10,000 Aim were determined. The magnetic properties were regarded as excellent if the respective magnetic flux densities were 1.20 T or more and 1.50 T or more.

Using a ring-shaped test piece having the same windings as above, the coercive force was measured with a reversal magnetization force of ±400 Aim using a DC magnetic property tester. The magnetic properties were regarded as excellent if the coercive force was 60 Aim or less.

### [Cold workability]

The cold workability was evaluated based on the critical upset ratio. In detail, a test piece of 15 mm in diameter and 22.5 mm in height and having a notch with a depth of 0.8 mm and a notch bottom radius R 0.15 on its side surface was collected from the depth position corresponding to 1/2 of the diameter from the peripheral surface of the steel bar. The test piece was subjected to compression forming. Compression was successively performed until a crack with a width of 0.5 mm or more occurred at the notch bottom of the test piece. The upset ratio at the time was taken to be the critical upset ratio.

The cold workability was regarded as excellent if the critical upset ratio was 55 % or more.

### [Machinability by cutting]

The machinability by cutting was evaluated by measuring the flank wear of the tool. In detail, using a NC lathe, the steel bar of 25 mm in diameter was subjected to cutting work with a cut depth of 0.2 mm, a feed rate of 0.15 mm/rev, a peripheral speed of 300 m/min, wet type, and a length of cut of 1000 m by a coating tool of cemented carbide. After this, the flank wear of the tool was measured to evaluate the machinability by cutting. The machinability by cutting was regarded as excellent if the flank wear was 35 µm or less.

## Claims

1. A soft magnetic iron comprising a chemical composition containing, in mass%,
C: 0.02 % or less,
Si: 0.15 % or less,
Mn: 0.01 % or more and 0.50 % or less,
P: 0.002 % or more and 0.020 % or less,
S: 0.001 % or more and 0.050 % or less,
Al: 0.05 % or less,
N: 0.0100 % or less, and
Se: 0.001 % or more and 0.30 % or less,
with a balance consisting of iron and inevitable impurities.

2. The soft magnetic iron according to claim 1, wherein the chemical composition further contains, in mass%, one or more selected from the group consisting of
Cu: 0.20 % or less,
Ni: 0.30 % or less,
Cr: 0.30 % or less,
Mo: 0.10 % or less,
V: 0.02 % or less,
Nb: 0.02 % or less, and
Ti: 0.03 % or less.

3. The soft magnetic iron according to claim 1 or 2, wherein the chemical composition further contains, in mass%, one or more selected from the group consisting of
Pb: 0.30 % or less,
Bi: 0.30 % or less,
Te: 0.30 % or less,
Ca: 0.0100 % or less,
Mg: 0.0100 % or less,
Zr: 0.200 % or less, and
REM: 0.0100 % or less.
